

## 1

3,825,424

### PROCESS FOR TRANSPARENT PHOTOGRAPHIC IMAGES

Robert F. Gracia, Scituate, Richard A. Laughrey,  
Woburn, and Paul F. Tuohey, Quincy, Mass., assignors  
to Itek Corporation, Lexington, Mass.

No Drawing. Application Oct. 1, 1969, Ser. No. 862,912,  
which is a continuation-in-part of application Ser. No.  
744,631, July 15, 1968, both now abandoned. Divided  
and this application Aug. 7, 1972, Ser. No. 278,310

Int. Cl. G03c 5/24

U.S. CL. 96—48 PD

21 Claims

#### ABSTRACT OF THE DISCLOSURE

This invention is concerned with a process of producing photographic images on a transparent substrate by photoexposure of a photographic medium of which the photosensitive layer is removable followed by prolonged treatment of the exposed medium to form a metal image adherently bonded to the substrate and subsequent removal of the photosensitive layer to obtain the metal image on the substrate, as well as the products produced thereby.

This case is a division of Ser. No. 862,912, filed Oct. 1, 1969, now abandoned, which is a continuation-in-part of U.S. Ser. No. 744,631, filed July 15, 1968, now abandoned.

#### BACKGROUND OF THE INVENTION

##### Field of the Invention

This invention relates to developed photographic media and processes for their production.

##### Description of the Prior Art

In the process of producing photographic images in transparent films, one of the difficulties encountered is the fog level which can develop in the photosensitive layer during photoprocessing. The development of fog in this layer necessitates special care and control in not only photographic development of the latent image but also in the selection and preparation of the photosensitive layer on the film in the production hereof. Such steps and precautions as are necessary to minimize fog, e.g. background density, in transparent films are well known to those skilled in the art and should not require extensive documentation for the purpose of this disclosure. In transparent films in which the photosensitive material is a photoconductor, e.g. titanium dioxide, care must be exercised to avoid the milky background of such films during development, which, though not always a significant problem, is met with some regularity in certain situations.

#### SUMMARY OF THE INVENTION

This invention relates to the process of producing photographic images on a transparent substrate by photoexposing a photographic medium comprising a removable photosensitive layer comprised of photosensitive material on a transparent support, contacting the photo-exposed medium with suitable image-forming material preferably a physical developer, to form a metal image in the exposed areas of the medium, prolonging the step of contacting with the image-forming materials until the formed metal image is adherently bonded to the support, and finally removing the photosensitive layer to obtain the metal image

## 2

on the support. The medium for use in the present process preferably includes a transparent substrate one face of which is superficially roughened and on which the photosensitive layer is applied. A preferred process is one utilizing a copy medium capable of being rapidly processed and having a very thin layer of a removable photosensitive layer on a superficially roughened transparent support. The rapid processing intended refers to contacting the copy medium with room temperature chemicals, such as silver nitrate and a reducing agent therefor, to produce an image adherently bonded to the support usually in less than about one minute.

#### DESCRIPTION OF PREFERRED EMBODIMENTS

The production of a photographic metal image which is adherent to the transparent substrate is accomplished by physical development of the exposed medium. The extent of such development required to obtain an image adherently bonded to the support is determined by many factors such as the intensity of light used during exposure, the concentration and type of reagents which make up the physical developer system, the time of development, and similar such considerations which are well understood by those skilled in photographic chemistry. A minimum of routine experimentation will permit the selection of proper reagents and conditions to obtain a metal image adherently bound to the substrate. For example, test strips of selected media can be exposed, developed and then subjected to treatment for removal of the photosensitive layer and the optimum conditions are thus determinable.

The photosensitive material of the present media can be any of those which permit physical development of a metal image, i.e. physically developable photosensitive materials. This type of photosensitive material is known in the art and embraces those photosensitive materials which after photoexposure are developable by what is known as physical development. Physical development is development using a solution of reducible metal ions and a reducing agent therefor which will selectively deposit metal in the photo-activated areas. In theory, the first step of such development is the formation of a latent metal image which is then intensified, or amplified, by the metal obtained by reduction of the aforesaid metal ions. The metal of the latent metal image may be the same as the so-reduced metal or different, e.g., the latent image can be silver and the so-reduced metal, copper or silver, as desired. In silver halide photography, the latent silver image forms in the silver halide emulsion and physical development is used to render the photo-image visible. Conveniently, the reducible metal ion for silver halide film is already present in the photosensitive emulsion in the form of the silver halide. However, an external source of reducible metal ion can be used in lieu thereof. Suitable photosensitive materials include silver halides, such as silver chloride or bromide; azo compounds, e.g. as described in British Specification 1,064,726, among others; photoconductors, as described in British Specification 1,043,250; ferric compounds; and methylene blue.

A physically-developed image can be:

- (1) the image formed on photoexposure, e.g. the latent silver image in silver halide emulsions or the reversible latent image on a photoconductor;
- (2) the irreversible image formed by contacting an exposed photoconductor-bearing medium with a sensitiz-

ing metal ion, e.g. a solution of silver ion, which can lead to an invisible irreversible image or a visible metal image;

- (3) the latent ferrous ion image formed by photoexposure of a ferric salt-sensitized medium and then sensitized with silver ion solution to form a silver image; or
- (4) a conductive image in close proximity but spaced from the support and which may be produced photographically, by printing, by writing or by physically placing a metallic image adjacent to the support.

Of the photosensitive materials, especially preferred are photoconductors, particularly as described hereinafter.

The preferred copy medium of this invention comprises a transparent base or support with the photosensitive material present in a layer of binder material. The copy medium especially preferred for use in this invention comprises a plastic base photographic plate capable of being stored in light or darkness without deterioration of its photosensitive components and capable further of being physically developed comprising a photoconductor which becomes reversibly activated upon exposure to activating radiation and is capable of causing chemical reaction in the exposed areas, this photoconductor preferably being deposited upon a superficially roughened support. The photoconductor is preferably of a particulate nature, preferably incorporated in a photoconductively insulating binder, and deposited as a very thin, removable layer upon the support, especially on a superficially roughened support, in such a way that the photoconductor is impregnated at least in part within the roughened surface of the support. This is readily accomplished for example by depositing a photoconductor, such as  $TiO_2$ , in a solvent-binder solution of relatively low viscosity and then coating this composition onto the roughened support. The coating composition may be allowed to dry. Such a support which has a photoconductor-binder coating will preferably have a very thin coating which is solvent permeable and will thereby allow rapid processing in the preferred developer systems.

The roughened support is a support which has been physically, chemically, or otherwise roughened in order that the metallic image forming materials are adherently bonded to the support. Physically roughened supports which are suitable for this invention are ones having grained, porous, or matted surfaces. Chemically roughened supports are ones which have been treated by suitable acids or bases, adhesive primers and the like to cause chemical bonding to take place between the image forming materials and the surface of the support. Additionally, additives such as cadmium and/or zinc salts may be added to the image forming materials in a manner such as described in French Patent of Addition No. 77,556 in order to improve the adhesion of the metal image to the support. The term "roughened supports," therefore, is intended to include a physically smooth support which by chemical or other means provides an adhesive bond with the metal image deposited thereon.

With supports comprising a plastic, i.e. a transparent plastic, the photosensitive layer is preferably coated on a subbed plastic sheet, such as sheets of a cellulose acetate, or a polyester, especially polyethylene terephthalate, containing a layer of material which improves the adhesion of the photosensitive layer to the plastic sheet. The intermediate layer is called a subbing layer, which concept is well known to the art. Usually, subbing layers comprise materials which adhere to the plastic material and to the more hydrophilic photosensitive layer. Generally, subbing layers are comprised of gelatin, but may also comprise various latex polymers, such as various vinylidene polymers, polyvinyl formals, polyvinyl butyral and similar such materials which are known in the art. The preferred subbing layers are those which imbibe the physical developer materials, for example, gelatins.

The thickness of the photosensitive layer or the image-forming layer, and the insulating layer or subbing layer, where present, will depend upon the nature of the photosensitive material, the nature of the binder, where present, the amount of activating radiation utilized, and other like factors. However, in order to obtain an imaging medium capable of rapid processing it is preferred that these layers be relatively thin, preferably less than about 50 microns in thickness. However, the thickness of the photosensitive layer and the insulating or subbing layer may vary within wide ranges. The coating thickness may be varied according to the effects desired. However, most preferable is a substrate wherein the coating is less than 10 microns in thickness in order to obtain the rapid processing which is most desired.

In general, the amount of binder to amount of photoconductor or other photosensitive material may vary over wide ranges. Preferably, from about 1 part by weight to about 6 parts by weight of photosensitive material per part by weight of binder will be used.

The photoconductor or photocatalyst preferred in this invention is a metal containing photoconductor. A preferred group of such photosensitive materials are the inorganic materials such as compounds of a metal and a non-metallic element of Group VIA of the periodic table such as oxides, such as zinc oxide,  $TiO_2$ , zirconium dioxide, germanium dioxide, indium trioxide; metal sulfides such as cadmium sulfide ( $CdS$ ), zinc sulfide ( $ZnS$ ) and tin disulfide ( $SnS_2$ ); metal selenides such as cadmium selenide ( $CdSe$ ). Metal oxides are especially preferred photoconductors of this group.  $TiO_2$  is a preferred metal oxide because of its unexpectedly good photosensitive properties.  $TiO_2$  having an average particle size less than about 250 millimicrons and which has been treated in an oxidizing atmosphere at a temperature exceeding about 200° C. is especially preferred, and more especially  $TiO_2$  produced by high temperature pyrolysis of titanium halide.

Organic photoconductors such as imidazolidinones and heteropolycacids mentioned in U.S. Ser. No. 623,534, now Pat. No. 3,623,865, incorporated herein by reference are also useful photosensitive materials in this invention.

Also useful in this invention as photoconductors are certain fluorescent materials. Such materials include, for example, compounds such as silver activated zinc sulfide, and zinc activated zinc oxide.

While the exact mechanism by which the photoconductors of this invention work is not known, it is believed that exposure of photoconductors or photocatalysts of this invention to activating means causes an electron or electrons to be transferred from the valence band of the photoconductor or photocatalyst to the conductance band of the same or at least to some similar excited state whereby the electron is loosely held, thereby changing the photoconductor from an inactive form to an active form. If the active form of the photoconductor or photocatalyst is in the presence of an electron accepting compound a transfer of electrons will take place between the photoconductor and the electron accepting compound, thereby reducing the electron accepting compound. Therefore, a simple test which may be used to determine whether or not materials have a photoconductor or photocatalytic effect is to mix the material in question with an aqueous solution of silver nitrate. Little, if any, reaction should take place in the absence of light. The mixture is then subjected to light. At the same time a control sample of an aqueous solution of silver nitrate alone is subjected to light, such as ultraviolet light. If the mixture darkens faster than the silver nitrate alone, that material is a photoconductor or photocatalyst.

It is evident that the gap between the valence and the conducting band of a compound determines the energy needed to make electron transitions. The more energy needed, the higher the frequency to which the photoconductor will respond. It is known to the art that it is possi-

ble to reduce the band-gap for these compounds by adding a foreign compound as an activator which either by virtue of its atomic dimensions or by possessing a particular electronic forbidden zone structure or through the presence of traps or donor levels in the intermediate zone between the valence and the conduction band stresses the electronic configuration of the photoconductive compound, thereby reducing its band-gap and thus increasing its ability to release electrons to its conduction band. Phosphors almost necessarily imply the presence of such activating substances. The effect of such impurities may be such as to confer photoconductivity upon a compound which intrinsically is non-photoconductive. On the other hand, excessive impurity content can interfere with a compound acting as a photoconductor, as above described.

The photoconductors may be sensitized to visible and other wavelengths of light by foreign ion doping, addition of fluorescent material, and/or by means of sensitizing dyes. Bleachable dyes useful for sensitizing the photoconductors include, for example, the cyanine dyes, the carbocyanine dyes, the carbocyanine dyes, and the hemicyanine dyes. Additional dyes which are useful for sensitizing the photoconductor are the cyanine dyes described on pages 371-429 in "The Theory of Photographic Process" by C. E. Kenneth Mees published by McMillan Company in 1952. Other useful dyes include those known to the art as triphenylmethane dyes such as crystal violet and basic Fuchsin, diphenylmethane dyes such as Auroamine O, and Xanthene dyes such as Rhodamine B.

The photosensitive material is used in a binder to form the photosensitive layer on the support, the sole requirement being that the layer be removable after photoprocessing. For removal, various methods can be used including dissolution or dispersion of the photosensitive layer using suitable liquid systems, such as solvents for the binder employed. Alternatively, removal of this layer with reactive solvents such as alkali or acid can be used, e.g. aqueous sodium carbonate, dilute sodium hydroxide, dilute phosphoric acid, phosphate salts and similar reagents. Mechanical removal of the photosensitive layer can be employed, e.g. using abrasive materials. Combinations of these methods can be used, e.g. rubbing the photosensitive layer from the support in the presence of a binder solvent or dispersing agent such as water. Other methods, e.g. gamma radiation of certain binders, can be used to render the layer frangible and it can then be removed mechanically.

Thus, the binders for use in the present media can comprise any of a wide variety of materials known in the photographic art. In general, these binders are translucent or transparent so as not to interfere with transmission of light therethrough. They are desirably also solvent permeable in order to allow rapid physical development to take place. Preferred binder materials are organic materials such as natural or synthetic polymers. Examples of suitable synthetic polymers are butadiene-styrene copolymer, poly(alkyl acrylates) such as poly(methyl methacrylate), polyamides such as polyacrylamide, polyvinyl acetate, polyvinyl alcohol and polyvinylpyrrolidone. Natural polymers such as gelatin are also useful. Most preferred are those binders which are solvent soluble enough to be readily washed off after development of the image has taken place. Preferably, for convenience the binder should be removable with aqueous systems. When not so removable, then suitable solvents which will dissolve or disperse the binder should be used. Little difficulty is encountered in selecting an appropriate solvent system since a simple solubility test can be used for the said purpose by merely immersing test media consisting of the support coated with the selected binder in various solvent systems. Solubility data for most binders are usually provided in standard texts or otherwise available. For example, methyl ethyl ketone, methyl isobutyl ketone, acetone, tetrahydrofuran, dioxane, and similar polymer solvents will be useful.

To obtain metal images according to this invention, the binder should not be removable by the photoprocessing conditions, i.e. the photosensitive layer should remain substantially intact during solution processing. However, if desired, binders which would dissolve in the processing solution during processing can be employed if viscous processing materials are employed, thus avoiding any substantial dissolution of the binder.

When employed as the photosensitive material, the photoconductor should be conditioned for exposure by storage in the dark from one to twenty-four hours prior to use, heating or other conditioning means known to the art. After conditioning the photoconductor is not exposed to activating radiation prior to its exposure to activating radiation for recording an image pattern.

The period of exposure to form the latent image will depend upon the intensity of the light source, particular photosensitive material, the type and amount of catalyst, if any, and like factors known to the art. In general, however, the exposure may vary from about 0.001 seconds to several minutes.

When the photosensitive material comprises a photoconductor, azo compounds, or ferric compounds, the physical developers according to this invention are intended to include those image forming systems such as described in U.S. Pat. 3,152,903, in British Patent Specification No. 1,043,250 and British Pat. 1,064,725. These image-forming materials include preferably an oxidizing agent and a reducing agent. Such image-forming materials are also often referred to in the art as electroless plating baths. Electrolytic development such as taught in U.S. Pat. 3,152,969 can also be used. The oxidizing agent is generally the image-forming component of the image-forming material. Either organic or inorganic oxidizing agents may be employed as the oxidizing component of the image-forming material. The oxidizing and reducing agent may be combined in a single processing bath, may also be in separate bath, or one or both of these components may be incorporated in the imaging medium prior to exposure. Preferred oxidizing agents comprise the reducible metal ions having at least the oxidizing power of cupric ion and include such metal ions as  $\text{Ag}^+$ ,  $\text{Hg}^{+2}$ ,  $\text{Pb}^{+4}$ ,  $\text{Au}^{+1}$ ,  $\text{Au}^{+3}$ ,  $\text{Pt}^{+2}$ ,  $\text{Pt}^{+4}$ ,  $\text{Ni}^{+2}$ ,  $\text{Sn}^{+2}$ ,  $\text{Pb}^{+2}$ ,  $\text{Cu}^{+1}$ , and  $\text{Cu}^{+2}$ .

When the photosensitive material comprises a silver halide, the physical developers can comprise a solution of an amplifying metal ion, e.g. silver, copper, tin and like ions with a reducing agent therefor, or the physical developer can comprise a silver reducing agent and a solvent for the silver halide. The silver halide solvents are well known in the photographic art and include any substance which will dissolve the unexposed silver halide of the photosensitive layer to form a solution thereof which functions as an amplifying agent for the latent image formed by the photoexposed silver halide. Commonly employed as silver halide solvents are soluble thiosulfate and thiocyanate salts, but any salt capable of dissolving silver halide, usually by complex ion formation, can be used for the same purpose as long as the complex ion formed is not of a high order of stability, i.e. not appreciably dissociated.

The reducing agent component of the said image-forming materials are inorganic compounds such as the oxalates, formates, and ethylenediaminetetraacetate complexes of metals having variable valence; and organic compounds such as dihydroxybenzenes, aminophenols, and aminoanilines. Also, polyvinylpyrrolidone, hydrazine, and ascorbic acid may be used as reducing agents in this invention. Suitable specific reducing compounds include hydroquinone or derivatives thereof, o- and p-aminophenol, p-methylaminophenol sulfate, p-hydroxyphenyl glycine, o- and p-phenylenediamine, 1-phenyl-3-pyrazolidone, alkali and alkaline earth metal oxalates and formates.

Liquid physical developer systems are preferred for use as image-forming materials because of the excellent

results obtained therewith. Any suitable solvent may be utilized. However, aqueous processing baths are preferred. While the pH of the developer is not critical, it has been found that the best results are obtained with an acid developer, and especially one having a pH of between about 2 and 5, and especially with organic acids such as citric, gluconic, maleic, and oxalic which are metal complexing agents. A pH of about 2 to 3 is especially preferred.

Additionally, the image-forming materials or physical developers may contain organic acids or alkali metal salts thereof, which can react with metal ions to form complex metal anions. Further, the developers may contain other complexing agents and the like to improve image formation and other properties found to be desirable in this art.

Additional developer systems useful in this invention are those disclosed in the following U.S. Patent Applications filed on July 11, 1968: Ser. No. 743,981, now Pat. No. 3,674,489, Ser. No. 743,982, now abandoned, and Ser. No. 743,983, now Pat. No. 3,645,736, each of which are incorporated herein by reference.

The physical developers of this invention should be applied for a length of time sufficient to obtain an image adherently bound to the support. This time period will vary according to the thickness of the photoconductor layer or thickness of the insulating layer or other separation layers, the length of exposure, nature of the binder or insulator material, ratio of photosensitive material to binder, and like factors known to the art.

The following examples are given to further illustrate the invention:

#### EXAMPLE 1

A layer of titanium dioxide in polyvinyl alcohol is coated on a gelatin-nitrocellulose subbed cellulose triacetate sheet, the gel-subbing serving as the hydrophilic subbing and the polyvinyl alcohol layer as the easily removed layer.

The coated sheets are exposed through a negative to a quartz-iodide lamp at 3 feet for 0.5 seconds and then processed by immersion for 10 seconds in 3 M  $\text{AgNO}_3$  (aqueous) followed by 20 seconds in a saturated solution of Metol containing 80 g./l. of citric acid monohydrate.

Gentle rubbing under a stream of running water removed the polyvinyl alcohol layer and a silver image is left in the gel-subbing layer. The result is a silver image on a transparent background.

Similar results are obtained when the photosensitive material is a ferric compound, azo compound or silver halide in a binder to form a removable layer.

When the triacetate sheet is replaced by a polyethylene terephthalate sheet, almost identical results are obtained.

This same procedure is used with a surface roughened polyethylene terephthalate sheet coated on the roughened side with the photosensitive layer without a subbing layer to obtain the silver image in the roughened surface of the sheet after removal of the developed photosensitive layer. The surface of the sheet is roughened by rubbing with an abrasive material.

#### EXAMPLE 2

A cellulose triacetate sheet with a roughened surface is coated with a layer of photosensitive silver bromide in polyvinyl alcohol exposed through a negative to actinic light and developed in a solution of hydroquinone containing 60 g./l. of sodium thiosulfate.

The polyvinyl alcohol layer is removed as in the preceding example to obtain a silver image in the roughened surface of the sheet.

#### EXAMPLE 3

A titanium dioxide coating, in which the pigment-binder ratio of titanium dioxide to polyvinyl alcohol is

6-1 and the total solids is 8%, is coated on a gelatin-nitro cellulose subbed film. The coating is applied with a No. 4 Meyer rod, or the coating can be applied via a dip technique. The coated sheet is then exposed in a conventional way and developed in the following bath for 90 seconds:

Solution I: G.  
 $\text{Fe}(\text{SO}_4)_2 \cdot (\text{NH}_4)_2 \cdot 6\text{H}_2\text{O}$  ----- 78.4  
 $\text{Fe}(\text{NO}_3)_3 \cdot 9\text{H}_2\text{O}$  ----- 33.2  
 Tartaric acid ----- 80.0  
 Distilled  $\text{H}_2\text{O}$  to 1 l.

Solution II: 10  
 Armac 12D ----- 1.0  
 Lissapol N ----- 1.0  
 Distilled  $\text{H}_2\text{O}$  to 1 l.

Solution III: 15  
 3 N  $\text{AgNO}_3$ .

The bath is made up in the following ratio: 20  
 Solution I ----- 125  
 Solution II ----- 25  
 Solution III ----- 6

The coating is then removed by gentle rubbing of the 25 surface. A diffused image remains in the subbing layer.

#### EXAMPLE 4

A titanium dioxide coating as described in Example 3 is coated on a subbed film and the subsequently exposed film is developed in the following solution:

Solution I: G.  
 Metol ----- 130  
 Citric acid ----- 180

Solution II: 35  
 3 N  $\text{AgNO}_3$ .

<sup>1</sup> To 1 liter.

150 cc. of Solution I are mixed with 5 cc. of Solution II just prior to development. The exposed film is developed for 90 seconds. The top coating is removed and a diffused silver image remains on the substrate.

#### EXAMPLE 5

45 A subbed polyester film base is coated with a finely divided titanium dioxide pigment dispersed in a polyvinyl alcohol binder. The pigment to binder ratio on a weight basis is 3:1 and the total solids of the emulsion is 15% by weight. The film base is coated on a roller coater yielding approximately 0.40 grams of titanium dioxide per square meter. The coated film is then dried and exposed with a quartz iodine lamp at a distance of 30 inches from the target through a vacuum printing frame for 2 seconds. After 10 seconds from the exposure the 50 sample is processed with a stabilized physical developer for 3 minutes. The physical developer is of the following formulation:

Solution I: G.  
 $\text{Fe}(\text{NH}_4)_2(\text{SO}_4)_2 \cdot 6\text{H}_2\text{O}$  ----- 78.4  
 $\text{Fe}(\text{NO}_3)_3 \cdot 9\text{H}_2\text{O}$  ----- 25.2  
 Tartaric acid ----- 80.0  
 $\text{H}_2\text{O}$  to 1 liter.

Solution II: 60  
 Armac 12D (ionic surfactant) ----- 1.0  
 Synthrapol N (nonionic surfactant) ----- 1.0  
 $\text{H}_2\text{O}$  to 1 liter.

Solution III: 65  
 $\text{AgNO}_3$  ----- 51.0  
 $\text{H}_2\text{O}$  to 100 ml.

The bath is made up in the following ratio: 70  
 Solution I ----- 250  
 Solution II ----- 50  
 Solution III ----- 6

The developed film is then placed in a tray of water at room temperature and wiped with a soft cotton pad to remove the coating. The resulting clear transparency has a maximum optical density of about 3.0. The image adhesion is tested by placing a strip of "Scotch Brand" tape over it and removing the tape with a quick pull. No silver is removed from the image area by this test. One sample of the processed film is contacted with an oleophilic lacquer which makes the film suitable for use as a lithographic master. A second sample in the form of a movie film strip with a variable area sound track adjacent to the photographic images is amplified with a nickel electroless plating solution in a manner such as described in the patent application filed on even date entitled "Photographically Prepared Magnetic Information Storage Element" by Laura Case. The photographic images on the movie film strip are of continuous tone and the variable area soundtrack can be read out with an ordinary magnetic reading head.

#### EXAMPLE 6

A layer of silver chloride in polyvinyl alcohol is coated on a subbed triacetate, the coating acting as an easily removed layer. The silver halide emulsion is made up in the following manner:

#### SILVER HALIDE EMULSION

##### Component I:

|                  |       |    |      |
|------------------|-------|----|------|
| NaCl             | ----- | g  | 0.50 |
| H <sub>2</sub> O | ----- | cc | 50.0 |
| 10% Lemol 16-98  | ----- | g  | 2.0  |

##### Component II:

|                       |       |    |      |
|-----------------------|-------|----|------|
| 3 N AgNO <sub>3</sub> | ----- | cc | 3.0  |
| H <sub>2</sub> O      | ----- | cc | 50.0 |
| 10% Lemol 16-98       | ----- | g  | 2.0  |

Component II is poured into Component I rapidly while stirring. A milky white emulsion of very fine particle size results. The emulsion is then sonified for four minutes on a Bronson sonifier, coated on a film base with a No. 4 Meyer rod, after which the coating is dried at 70° F. for five minutes. It is then exposed in a conventional manner and processed in any of the physical developers described in the other examples. The top is removed and a diffused image results in the subbed layer. Thus, an imaged film with excellent transparency is produced.

The same results are obtained using a polyester film in lieu of cellulose acetate film.

In the foregoing examples, the final products consist of the developed metal image on the transparent substrate. These products are especially suitable for photocopying and projection, e.g. projection slides. Further treatment of these products by conventional methods converts them into printing masters, e.g. increasing the oleophilic nature of the metal image on a comparatively hydrophilic substrate renders the images ink receptive. Thus, the metal images can be treated with mercaptans and/or lacquered by art-recognized procedures commonly employed in preparing printing plates and then inked and used as a printing master.

The present invention can also be employed in the formation of printed electrical circuits and the metal circuit is obtained on the transparent support. The metal circuit can be further amplified with a desired metal, e.g. copper, using standard procedures including electrolytic plating and electroless plating by art-recognized procedures. The initially developed metal circuit is comprised of a continuous, electrically-conductive metal image which is formed of large, contiguous particles of the metal which gives the appearance of a continuous layer. This form of

image is preferred for use in printing masters and in printed electrical circuits.

In the foregoing examples, little if any special care has to be observed regarding fog development in the photosensitive layer since the photosensitive layer is subsequently removed. After removal of the photosensitive layer, the final products retain the original transparency of the substrate.

The term "pellucid" as used herein is intended to mean transparent or translucent. The above description while using the term "transparent" is intended to include a "pellucid" copy medium.

What is claimed is:

1. A process of producing a photographic metal image on a roughened pellucid support therefor which comprises the steps of:

- (a) exposing a copy medium comprising a thin removable layer comprised of photosensitive material in a binder therefor on a pellucid support to form a physically developable image in said medium;
- (b) physically developing by contacting the exposed medium with image-forming material comprising a solution of metal ions to form a metal image in the exposed areas of the medium;
- (c) prolonging the step of contacting with the image-forming materials until the formed metal image is adherently bonded directly to the support; and
- (d) removing the photosensitive layer and leaving the metal image on the support.

2. Process as in Claim 1 wherein the removable layer comprises a solvent-removable binder for the photosensitive material.

3. Process as in Claim 1 wherein the support is a subbed plastic sheet.

4. Process as in Claim 3 wherein the plastic is a cellulose acetate.

5. Process as in Claim 3 wherein the plastic is a polyester.

6. Process as in Claim 3 wherein the plastic is polyethylene terephthalate.

7. Process as in Claim 3 wherein the subbed sheet is a gelatin-subbed sheet.

8. Process as in Claim 1 wherein the photosensitive material comprises a photoconductor.

9. Process as in Claim 1 wherein the photosensitive material comprises a photosensitive silver halide.

10. A process of producing a photographic metal image on a pellucid support therefor which comprises the steps of:

- (a) exposing a copy medium comprising a thin removable layer comprised of titanium dioxide in a binder therefor on a pellucid support to form a physically developable medium in said medium;
- (b) contacting the photo-exposed medium with a physical developer comprising a solution of reducible metal ions to form a metal image in the exposed areas of the medium;
- (c) prolonging the step of contacting with the image-forming materials until the formed metal image is adherently bonded directly to the support; and
- (d) removing the titanium dioxide layer and leaving the metal image on the support.

11. Process as in Claim 10 wherein the removable layer comprises a solvent-removable binder for the photosensitive material.

12. Process as in Claim 10 wherein the support is a subbed plastic sheet.

13. Process as in Claim 10 wherein the plastic is a cellulose acetate.

14. Process as in Claim 10 wherein the plastic is a polyester.

15. Process as in Claim 10 wherein the plastic is polyethylene terephthalate.

16. Process as in Claim 10 wherein the subbed sheet is a gelatin-subbed sheet.

17. Process as in Claim 10 wherein the reducible metal ions are silver ions.

18. Process as in Claim 10 wherein the physical developer comprises a reducing agent for the metal ions.

19. Process as in Claim 18 wherein the metal is silver 5 or copper.

20. Process as in Claim 10 including the further step of amplifying the metal image after removal of the titanium dioxide layer.

21. Process as in Claim 20 wherein the amplifying step is accomplished with a silver, copper or tin ion solution including a reducing agent for the selected metal ions.

## UNITED STATES PATENTS

|           |         |              |       |          |
|-----------|---------|--------------|-------|----------|
| 3,149,970 | 9/1964  | Weyde        | ----- | 96-48 PO |
| 3,674,489 | 7/1972  | Wyman et al. | ----- | 96-48 PO |
| 3,409,429 | 11/1968 | Ekman et al. | ----- | 96-48 PO |
| 3,152,903 | 10/1964 | Shephard     | ----- | 96-64    |

RONALD H. SMITH, Primary Examiner

10 E. C. KIMLIN, Assistant Examiner

U.S. Cl. X.R.

96-1 R, 1.5, 1.8, 87 R